

1

3,082,156

## NICKEL PLATING ON ZINC

Richard C. Brown, Muncie, Ind., assignor, by mesne assignments, to American Zinc Institute Incorporated, New York, N.Y., a corporation of New York  
No Drawing. Filed Aug. 19, 1960, Ser. No. 50,607  
4 Claims. (Cl. 204—49)

This invention relates to nickel plating, and particularly to a method and composition for electroplating nickel directly on zinc and zinc base alloys.

Plating directly on zinc and zinc base alloys with nickel strike baths of the present invention eliminates copper plating in a cyanide bath, prevents formation of a brittle intermetallic copper-zinc phase, and improves corrosion resistance of die castings, which may be further plated with nickel or chromium.

In the past, it has been customary to plate copper on zinc and zinc base alloys in a cyanide bath before applying a bright nickel plate or a chromium plate. The copper cyanide baths are toxic, and it is necessary to treat plating room wastes carefully and completely when such baths are used. This is a costly operation that the plating industry is seeking to avoid. Another disadvantage is that brittle intermetallic copper-zinc compounds are formed at ambient temperatures by diffusion between the die-cast, zinc alloy basis metal and the copper plate. The diffusion alloying often causes blistering or peeling of the electroplate and leads to unsatisfactory appearance. The baths for the present invention are not toxic, and the nickel strike process of this invention does not cause any brittle compounds or alloys to form. The invention improves corrosion resistance and provides a very strong bond between the electroplate and the basis metal.

Various attempts to develop nickel plating baths for plating directly on zinc have been unsuccessful. Of the baths described in the prior art, one used nickel chloride, tartaric acid, and ammonium hydroxide (to adjust the pH to 5.6). Only porous, black deposits with poor covering power were obtained using this bath in the manner taught. In another bath, additions of sodium citrate, disodium dihydrogen, ethylene-diaminetetra acetic acid, triethanol amine, sodium sulfate, and sodium hydroxide were made to nickel sulfate solutions. Only porous, cracked deposits were obtained in plating directly on zinc die castings. A nickel phosphate-phosphoric acid bath described in the literature proved to be unsuitable for plating on zinc die castings. A bath containing nickel sulfate, sodium citrate, ammonium hydroxide, and sodium pyrophosphate provided a dense plate, but the plate was inferior in adherence.

The nickel plate obtained on zinc and zinc alloys with baths containing chloride or other halide ions is porous, because the halide ion tends to dissolve the zinc or alloy; and the adherence of the plate is poor. Without the halide in the conventional nickel sulfate bath, dissolution of the nickel anodes is not sufficient for satisfactorily replenishing nickel ions in the plating bath. Replacing the halide ions with fluoborate and citrate ions in accordance with the present invention, however, enables satisfactory anode dissolution and a superior plate.

Baths containing only nickel sulfate and nickel fluoborate provide deposits that are generally satisfactory except for areas of low current density, which remain unplated. To improve the throwing power, it has been common to add salts of organic acids as the potassium or sodium salt. Materials such as sodium and potassium citrates and tartrates improve the throwing power of the nickel deposited in the sulfate fluoborate bath, but these additions cause the electroplate to be porous. In the present invention it has been found that substituting nickel

2

citrate for a part of the nickel sulfate improves the throwing power of nickel sulfate-nickel fluoborate baths without causing the electroplate to be porous.

The table below lists preferred and useful ranges of bath compositions and operating conditions for nickel strike plating directly on zinc and zinc base alloys according to the present invention.

TABLE

|                                                                 | Preferred Range                     | Useful Range                        |
|-----------------------------------------------------------------|-------------------------------------|-------------------------------------|
| Bath Constituents:                                              |                                     |                                     |
| Nickel Sulfate, $\text{NiSO}_4 \cdot 7\text{H}_2\text{O}$       | 1.0 to 1.2 molar                    | 0.5 to 1.5 molar                    |
| Nickel Fluoborate, $\text{Ni}(\text{BF}_4)_2$                   | 0.2 to 0.3 molar                    | 0.1 to 0.4 molar                    |
| Nickel Citrate, $\text{Ni}_3(\text{C}_6\text{H}_5\text{O}_7)_2$ | 0.07 to 0.15 molar                  | 0.05 to 0.2 molar                   |
| Boric Acid, $\text{H}_3\text{BO}_3$                             | 0.3 to 0.5 molar                    | 0.1 molar to saturation             |
| pH                                                              | 4.5 to 4.9                          | 3.5 to 5.5                          |
| Operating Conditions:                                           |                                     |                                     |
| Temperature                                                     | 65 to 75 F.                         | 60 to 85 F.                         |
| Cathode current density                                         | 75 to 125 amp./sq. ft.              | 50 to 200 amp./sq. ft.              |
| Work bar agitation                                              | 25 to 60 c.p.m.; 2 to 4 inch stroke | 15 to 70 c.p.m.; 1 to 6 inch stroke |
| Air agitation                                                   | Optional                            | 5 to 75 amp./sq. ft.                |
| Anode current density                                           | 10 to 40 amp./sq. ft.               |                                     |
| Voltage (between anode and cathode)                             | 4 to 7 volts                        | 3 to 12 volts                       |
| Plating time                                                    | 1 to 5 minutes                      | 1 to 10 min.                        |
| Plating rate                                                    | 0.003 to 0.005 inch/hour            | 0.002 to 0.008 inch/hour            |
| Thickness of deposit                                            | 0.00005 to 0.00015 inch             | 0.00005 to 0.0005 inch              |

In a typical operation of nickel strike plating on an item made of zinc or a zinc base alloy according to the present invention, the item to be plated is either buffed or electropolished, and degreased in trichloroethylene, or electropolished after degreasing. It is then cleaned conventionally either anodically or cathodically, but preferably anodically, and rinsed in hot and cold water, acid dipped in 0.25 to 1.0 (weight) percent sulfuric acid solution, and rinsed in cold water. The item is then immersed in the plating bath and the work bar is started. With an appropriate D.C. power supply to provide the desired current density, the circuit is closed to start electrodeposition. The plating is continued for the desired period, after which the circuit is opened, the work bar is stopped, and the plated item is removed and rinsed.

Among the advantages of the present invention are: simplicity of composition, better appearance, less porosity, better bond to basis metal, better covering in low current density areas, and less tendency to crack or flake.

The following examples show some of the advantageous results obtained with the present invention:

### Example I

Buffed and cleaned zinc alloy (AG40-A, also known as Zamak 3) were plated directly in an aqueous plating bath containing:

|                                                                 |                |           |
|-----------------------------------------------------------------|----------------|-----------|
| Nickel sulfate, $\text{NiSO}_4 \cdot 7\text{H}_2\text{O}$       | — molar        | 1.14      |
| Nickel fluoborate, $\text{Ni}(\text{BF}_4)_2$                   | — do —         | 0.28      |
| Nickel citrate, $\text{Ni}_3(\text{C}_6\text{H}_5\text{O}_7)_2$ | — do —         | 0.08      |
| Boric acid, $\text{H}_3\text{BO}_3$                             | — do —         | 0.4       |
| pH                                                              | —              | 4.9 ± 0.2 |
| Temperature                                                     | — ° F.         | 74 ± 2    |
| Cathode current density                                         | — amp./sq. ft. | 100       |

Approximately 0.0001 inch of smooth, fine-grained, gray nickel was deposited adherently in 1.5 to 1.75 minutes with a cathode current efficiency of 93 percent. Low-current-density (recessed) areas were covered adequately with a uniform appearance, free of pits or other defects. After rinsing, the nickel-plated die castings were plated with bright nickel in a Watts type nickel bath containing

known brighteners. In five minutes, smooth, mirror like nickel plate was deposited about 0.0003 inch thick.

*Example II*

Because thicker deposits of bright nickel, i.e. 0.001 inch, or more, were brittle and showed a little cracking at edges of complex-shaped parts previously plated with 0.0001 to 0.0002 inch of nickel in the sulfate-fluoborate-citrate bath, an intermediate nickel plate was deposited prior to bright nickel, when a total nickel thickness of 0.001 inch, or more, was desired. By this procedure, zinc die castings first nickel plated by the procedure of Example I were next plated with additional nickel in one of the two following solutions:

*Example IIa (Watts-Type Bath)*

|                                                            |       |               |
|------------------------------------------------------------|-------|---------------|
| Nickel sulfate, $\text{NiSO}_4 \cdot 7\text{H}_2\text{O}$  | molar | 1.5           |
| Nickel chloride, $\text{NiCl}_2 \cdot 6\text{H}_2\text{O}$ | do    | 0.2           |
| Boric acid, $\text{H}_3\text{BO}_3$                        | do    | 0.6           |
| pH                                                         |       | $3.7 \pm 0.2$ |
| Temperature                                                | ° F.  | $135 \pm 3$   |

*Example IIb*

|                                                         |       |               |
|---------------------------------------------------------|-------|---------------|
| Nickel sulfamate, $\text{Ni}(\text{H}_2\text{NSO}_3)_2$ | molar | 1.8           |
| Boric acid, $\text{H}_3\text{BO}_3$                     | do    | 0.5           |
| pH                                                      |       | $5.0 \pm 0.2$ |
| Temperature                                             | ° F.  | 80 to 85      |

With a current density of 30 to 40 amp./sq. ft. in each case, approximately 0.0002 inch of gray nickel was deposited in 10 to 12 minutes. After rinsing, the parts next were plated with 0.0007 inch, or more, of bright nickel.

Die castings that were plated according to any of the above examples showed no evidence of blistering, peeling, or delamination when they were subjected to sawing, filing, hammering, or heating (to 325° F.). Metallographic examination of cross sections likewise showed no peeling or delamination.

What is claimed is:

1. A method of electroplating comprising plating nickel on zinc and zinc base alloys from an aqueous solution

consisting essentially of about 0.5 to 1.5 mols per liter of nickel sulfate, about 0.1 to 0.4 mol per liter of nickel fluoborate, about 0.05 to 0.2 mol per liter of nickel citrate, and about 0.1 mol per liter to saturation of boric acid, said solution having a pH from about 3.5 to 5.5 at a cathode current density of about 50 to 200 amperes per square foot, while maintaining the temperature of said solution between about 60 and 85° F.

2. A composition of matter for electroplating nickel on zinc and zinc base alloys consisting of an aqueous solution consisting essentially of about 0.5 to 1.5 mols per liter of nickel sulfate, about 0.1 to 0.4 mol per liter of nickel fluoborate, about 0.05 to 0.2 mol per liter of nickel citrate, and about 0.1 mol per liter to saturation of boric acid, said solution having a pH from about 3.5 to 5.5.

3. A method of electroplating comprising plating nickel on zinc and zinc base alloys from an aqueous solution consisting essentially of about 1.0 to 1.2 mols per liter of nickel sulfate, about 0.2 to 0.3 mol per liter of nickel fluoborate, about 0.07 to 0.15 mol per liter of nickel citrate, and about 0.3 to 0.5 mol per liter of boric acid, said solution having a pH from about 4.5 to 4.9 at a cathode current density of about 75 to 125 amperes per square foot, while maintaining the temperature of said solution between about 65 and 75° F.

4. A composition of matter for electroplating nickel on zinc and zinc base alloys consisting of an aqueous solution consisting essentially of about 1.0 to 1.2 mols per liter of nickel sulfate, about 0.2 to 0.3 mol per liter of nickel fluoborate, about 0.07 to 0.15 mol per liter of nickel citrate, and about 0.3 to 0.5 mol per liter of boric acid, said solution having a pH from about 4.5 to 4.9.

References Cited in the file of this patent

UNITED STATES PATENTS

|           |          |               |
|-----------|----------|---------------|
| 2,069,566 | Tuttle   | Feb. 2, 1937  |
| 2,539,588 | Moy      | Jan. 30, 1951 |
| 2,871,172 | Atkinson | Jan. 27, 1959 |
| 3,003,933 | Atkinson | Oct. 10, 1961 |